

# United States Patent Office

3,176,375

Patented Apr. 6, 1965

1

3,176,375

METHOD OF MAKING PAPER-MACHINE FELT  
Thomas Hindle and Edward Race, Blackburn, England,  
assignors to Scapa Dryers Ltd., a company of Great  
Britain, Northern Ireland, and the Isle of Man  
No Drawing. Original application Aug. 8, 1960, Ser. No.  
47,956. Divided and this application June 20, 1963,  
Ser. No. 289,381  
11 Claims. (Cl. 28--73)

This invention pertains to woven textile fabrics, in particular to a novel method of manufacturing fabric useful as a paper-machine felt such as is employed in the manufacture of pulp, paper, board, asbestos-cement sheets, pipes and similar or related products, the present application being a division of the copending application for Letters Patent, Serial No. 47,956, filed August 8, 1960, by Thomas Hindle and Edward Race.

According to customary, prior practice, these "felts" were manufactured entirely from wool yarns, or, particularly in the case of the felts used in the production of asbestos-cement products, from a combination of wool and cotton. With the advent of nylon, polyester and similar synthetic fibres, it was found that by manufacturing the felt from yarns composed of blends of wool fibres and synthetic fibres, the abrasion-resistance of the felts was greatly improved and the felts exhibited a longer service life.

Whenever a paper-machine felt is composed entirely of wool or a mixture of wool and synthetic fibres, milling or fulling is an essential operation in the manufacture of the felt. Thereby, the weave structure of the felt, which otherwise would mark the paper, is masked at the surface by the matted or felted wool fibres and yet its permeability to water remains of a high order.

Since conventional synthetic fibres do not possess the felting characteristics of most fibres, it was thought essential until recently that the proportion of synthetic fibres incorporated in a woven felt must be less than that which would prevent appreciable milling or fulling of the felt. However, it has been discovered recently that if such a "felt," made wholly or predominantly of synthetic fibres, has one or both of its surfaces raised, as by napping or gigging, and the raised fabric is subjected to a process of needling, the surface texture of the resultant fabric simulates closely enough to that of a milled felt made wholly or predominantly of wool to be used as a paper-machine felt. The operation of needling is effected in any known manner, as by passing the woven fabric through a machine wherein the surface of the fabric is frequently pierced by barbed needles, the result being to force the nap fibres constituting the raised surface into the body of the fabric.

Unfortunately, in many instances, prolonged needling is required in order effectively to entangle the raised fibres into the woven body of the fabric. Two major defects are liable to arise as a result of the prolonged needling operation. Firstly, serious reduction in the water permeability of the felt is possible, and it is not unusual for the water permeability of the felt after extensive needling to be only one-half of its initial value. This reduction in permeability has an adverse effect on the rate of drainage of water from the paper sheet through the felt when the latter is in operation on the paper-machine. Secondly, the process of prolonged needling the raised, woven fabric breaks many of the fibres both of the raised surface and of the yarns in the body of the felt. This weakens the fabric and makes it more susceptible to degradation by mechanical abrasion.

The expression "endless woven fabric" as used herein, is intended to include not only fabric which is woven endless initially (the weft in the loom becoming the warp in the finished fabric), but also a length of fabric, woven

2

flat, whose ends have been joined, and wherein the warps and wefts of the fabric are the loom warps and wefts. In this specification by the term "warp" is, therefore, meant those yarns arranged in the longitudinal direction of the endless finished product (regardless of how produced), such as a papermaker's dryer felt and by the term "weft" is meant those yarns arranged in a direction which is transverse of the length of the finished product. The synthetic content of the yarns may be in the form of a plurality of continuous filaments, or staple fibres thereof, and general references to "synthetic fibres" or "fibres" when they occur herein and in the claims hereof are intended to include, within their scope, both forms.

In felting wool, adjacent fibres become entangled one with another, and not only do fibres within the same yarn become entangled, but the surface fibres of one yarn become entangled with the surface fibres of adjacent yarns running parallel and with the surface fibres of yarns crossing one another. Thus, in wool felting, adjacent fibres become attached to one another, and yarns are likewise attached to each other at their crossing points. Broadly stated, the objects of the present invention provide a method of making a felt which has the wear resistance attributable to the incorporated synthetic but which also predominantly synthetic possesses the desirable characteristics of a felted wool felt.

In accordance with the method of the present invention the synthetic fibres and crossing yarns are joined together by integral bonds of the material of which they are composed.

A further object of the present invention is to provide a novel method of producing an adequately water-permeable woven fabric, for use as a paper-machine felt, which is wholly or predominantly of synthetic fibre and which has not been subjected to a needling or equivalent operation. Another object is to provide a method of making woven textile fabric sufficiently pervious to the passage of water and sufficiently flexible to function satisfactorily as a paper-machine felt and which consists, at least predominantly, of synthetic fibres and wherein, wherever constituent synthetic fibres touch one another, they are bonded together at their mutual points of contact, with the result that synthetic warp and weft yarns, whatever their individual character, become bonded together at their crossing points.

A further object is to provide a novel method of making woven textile fabric, sufficiently water-permeable to constitute a satisfactory paper-machine felt and which consists, at least predominantly, of synthetic fibres, which, 50 comprises the step, after weaving, of so treating the fabric as integrally to bond adjacent synthetic fibres at their crossing points.

A further object is to provide a novel method of making a woven textile fabric, adequately water-permeable for use as a paper-machine felt and which consists, at least predominantly, of synthetic fibres, which comprises so treating the fabric, after weaving, with a fluid reagent which acts preferentially at the points at which the fibres cross one another, as to cause the fibres to coalesce at 60 said points to form integral bonds.

Briefly stated the invention provides a novel method comprising as steps; providing a fabric wherein warps and wefts, predominantly of synthetic fibrous material, are so interwoven as to form a structure acceptable for use as the base fabric of a paper-machine felt, and thereafter subjecting said fabric to the action of a chemical reagent which causes some, at least, of the constituent synthetic fibres to coalesce at their mutual points of contact, whereby said contacting fibres are integrally and permanently bonded together. More specifically, the preferred method employs as a reagent an aqueous solution

of an inorganic salt which, in concentrated form, acts on some, at least, of the synthetic fibres to gel them so as to cause contacting fibres to coalesce and form integral bonds at their mutual points of contact, and thereafter washing the fabric to remove the salt, and drying the material.

Preferably the aqueous solution is caused to concentrate and to localize preferentially in the region of said points of contact, after application to the fabric.

In the case of fabrics made wholly or predominantly of nylon, which is a polyamide fibre, and/or acrylic fibres, such as Orlon (a registered trademark, the property of E. I. du Pont de Nemours & Co.) or Courtelle (a registered trademark, the property of Courtaulds Ltd.), (both being acrylic fibres such as those made of polyacrylonitrile and copolymers thereof) suitable salts are calcium and lithium bromides and calcium and magnesium thiocyanates. In the case of fabrics made wholly or predominantly of polyester fibres, such as Terylene (a registered trademark, the property of Imperial Chemical Industries Ltd.) or Dacron (a registered trademark, the property of E. I. du Pont de Nemours & Co.), or containing a material proportion of such fibres in addition to acrylic and/or polyamide fibres, suitable salts are calcium and magnesium thiocyanates.

In applying the invention, a woven fabric, made wholly or predominantly of synthetic fibres and suitable for use as a paper-machine or like felt, is impregnated with an aqueous solution of the selected salt and the water is evaporated from the fabric so that the salt solution concentrates. During concentration, the salt solution tends to localize preferentially at the crossover points of the fibres. As evaporation of the water continues, the salt solution ultimately becomes sufficiently concentrated to gelatinize small portions of the fibre surfaces at the crossover points, and on complete evaporation of the water, the fibres become bonded with adjacent fibres. Thereafter, the inorganic salt is washed out of the fabric with water.

If a woven fabric for use as a paper-machine felt is composed of a mixture of two synthetic fibrous materials, then a salt capable of swelling and dissolving or gelatinizing the surface of both fibres is employed. For example, if the fabric is composed of nylon and Terylene, then calcium or magnesium thiocyanate is employed as the reactant.

The concentration of inorganic salt in the impregnating liquor can be as low as 0.5% by weight, although for good fibre-to-fibre bonding, it is preferred that a 2% to 5% solution is used, and the solution can, in fact, have a concentration of inorganic reactant as high as 10% by weight.

One example of the processing according to the invention is as follows:

An endless woven fabric of a structure suitable for use as a paper-machine felt has warp and weft yarns spun from crimped nylon staple fibres. The fabric is treated at ambient temperature for 15 minutes in a 5% by weight solution of lithium bromide, 4 gallons of solution being used for every 10 lb. of synthetic fibre. The impregnated fabric is hydro-extracted and then dried on a felt-stretching machine, at least one cylinder of which is heated. As the water evaporates from the felt, thus concentrating the lithium bromide, the latter tends to collect at the fibre crossovers, gelatinisation of which results in fibre-to-fibre bonding. When the fabric is completely dry, it is washed in water until free from lithium bromide, hydro-extracted, and re-dried on the felt-stretching machine.

The above is only one method of carrying out the invention. Any conventional method of impregnation and drying can be used and the concentration and amount of reactant salt can be varied without departing from the invention.

Furthermore, the fabric need not necessarily be woven wholly from spun synthetic yarns and, as has been pointed

out hereinbefore, the general references to "synthetic fibres" and "fibres" herein and in the claims, are not intended to be limited to the fibres of such yarns. For example, the warp yarns may be spun from crimped synthetic fibres, or from straight synthetic staple fibres, or may be continuous filament synthetic yarns, or continuous filament bulked synthetic yarns of the non-stretch type, such as Taslan-textured yarns, or yarns composed of a core of continuous filament synthetic yarns around which is wrapped a finer Taslan-textured yarn. ("Taslan" is a trademark registered by E. I. du Pont de Nemours & Co.). The weft yarns are preferably spun from synthetic staple fibres, but these staple fibres may be the commercially-produced crimped synthetic fibres, or they may be prepared by cutting into staple fibre length those commercially-produced continuous filament yarns which are known as "bulked yarns" and "stretch yarns" and "bulked and stretch yarns."

While, in accordance with the present invention, the synthetic fibres are bonded together at their mutual points of contacts, it should be remembered that it is extremely rare to find two fibres in a spun yarn which make a line contact of appreciable length, although they may repeatedly cross each other, so that the practice of the present process does not result in stiffening or reducing the normal flexibility of the felt to a degree such as to impair its utility for the intended purpose.

Moreover, the present fibre-bonding process can be applied with advantage to the wholly or predominantly synthetic paper-machine felts, described in our copending United States application Serial No. 47,956, filed August 8, 1960, in which the weft yarns are spun from blends which contain shrinkable fibres.

With felts for use on certain types of paper-machines it is preferred to raise, as by napping, one or both surfaces of the woven fabric before impregnation with the reactant solution. In other instances, it is preferred first to bond the fibres by impregnation, evaporation of the entrained water and rewashing and thereafter to raise one or both surfaces. In this latter case, although the operation of raising breaks some of the bonds on the surface fibres, these fibres are still bonded below the raised surface, and the fibres of the yarns unaffected by raising are, of course, still bonded to one another. In either case, the nap fibres collectively mask the weave pattern and provide a smooth surface.

In cases where particularly good bonding is required, during the drying process following impregnation, the fabric can be pressed against the heated cylinder of the felt-stretching machine by means of a relatively heavy roller.

We claim:

1. The method of making a woven fabric suitable for use as a papermaker's felt and which possesses wear-resistance such as results from the incorporation therein of at least a predominance of synthetic fibrous material and which possesses desirable characteristics of a conventional wool felt, including flexibility and permeability to water, said method comprising the steps of providing woven fabric, of a structure acceptable for use as a base fabric of a papermaker's felt and consisting, at least in major proportion, of synthetic fibres, impregnating the fabric with a weak aqueous solution of inorganic salt, progressively concentrating the salt solution, thereby intensifying the normal tendency of the solution to migrate toward and accumulate at the points at which fibres cross and contact one another, whereby the concentrated salt solution reacts with the fibres at said crossing points, causing them to gel and coalesce and to form permanent bonds predominantly at the fibre crossing points, whereby the fabric retains an acceptable percentage of its initial water-permeability and flexibility, then washing the fabric to remove the salt, and thereafter drying the fabric.
2. The method according to claim 1, wherein the initial concentration of the aqueous salt solution is between 2% and 10% by weight.

3. The method according to claim 1, wherein the inorganic salt is selected from the group consisting of calcium bromide and lithium bromide.

4. The method according to claim 1, wherein the inorganic salt is selected from the group consisting of calcium thiocyanate and magnesium thiocyanate.

5. The method according to claim 1, wherein the fabric consists, at least predominantly, of polyester synthetic fibres, and wherein the inorganic salt is selected from the group consisting of calcium thiocyanate and magnesium thiocyanate.

6. The method according to claim 5, wherein the fabric includes a substantial proportion of polyamide fibre.

7. The method according to claim 5, wherein the fabric comprises a substantial proportion of acrylic fibre.

8. The method according to claim 1, wherein the fabric is predominantly of polyamide fibre and the inorganic salt is selected from the group consisting of calcium bromide, lithium bromide, calcium thiocyanate and magnesium thiocyanate.

9. The method according to claim 1, wherein the fabric consists predominantly of acrylic fibre and the inorganic salt is selected from the group consisting of calcium bromide, lithium bromide, calcium thiocyanate and magnesium thiocyanate.

25

10. The method according to claim 1, further characterized in napping one side, at least, of the material after it has been dried.

11. The method according to claim 1, wherein one, at least, of the faces of the woven fabric is napped, prior to impregnation with the salt solution.

#### References Cited by the Examiner

##### UNITED STATES PATENTS

|    |           |       |                |         |
|----|-----------|-------|----------------|---------|
| 10 | 2,255,890 | 9/41  | Knowland       | 28—73   |
|    | 2,332,373 | 10/43 | Dorough et al. | 28—73   |
|    | 2,365,931 | 12/44 | Benger         | 28—1    |
|    | 2,389,120 | 11/45 | Castellan      | 28—73   |
|    | 2,392,842 | 1/46  | Doell          | 57—157  |
| 15 | 2,401,291 | 5/46  | Smith          | 57—140  |
|    | 2,460,674 | 2/49  | Bihaly         | 28—73   |
|    | 2,465,996 | 4/49  | Bloch          | 28—1    |
|    | 2,771,659 | 11/56 | Ball           | 28—73   |
| 20 | 2,811,029 | 10/57 | Conner         | 28—73   |
|    | 2,903,021 | 9/59  | Holden et al.  | 139—426 |

DONALD W. PARKER, *Primary Examiner.*

MERVIN STEIN, *Examiner.*

25